

# United States Patent Office

2,992,920

Patented July 18, 1961

1

2,992,920

## PRODUCTION OF COLORED PHOTOGRAPHIC IMAGES

Arthur Henri De Cat, Antwerp, and Bernard Hippoliet Tavernier, Mortsel-Antwerp, Belgium, assignors to Gevaert Photo-Producten N.V., Mortsel, Belgium, a Belgian company

No Drawing. Filed Mar. 10, 1958, Ser. No. 720,013  
Claims priority, application Great Britain Mar. 15, 1957  
4 Claims. (Cl. 96—55)

The present invention relates to a process for the manufacture of colored photographic images by color development in the presence of a color coupler, to photographic developers which contain such color coupler and to photographic images obtained according to this process.

It is known to obtain a colored photographic image by developing a reducible silver salt image in the presence of a color coupler, i.e. a compound which during development couples with the oxidation product of the developing agent and forms a dyestuff which precipitates onto the developed silver grains.

Yellow colored images are usually obtained by development in the presence of compounds which contain an active methylene group, particularly acylacetanilide derivatives.

It is an object of the present invention to provide a new process of color development. It is another object of the present invention to provide new photographic developers. It is a further object of the present invention to provide new colored photographic images. Still further objects will appear from the following description.

These objects are accomplished by the use as color couplers of a class of compounds, some members of which are preferable to the known compounds by combining high solubility in the developer, insolubility of the resulting dyestuffs which do not bleed out and moreover greater activity than is found with other acylacetanilides.

According to the present invention, a reducible silver salt image is developed with an aromatic amino developing agent in the presence of a compound according to the formula:



wherein

Y=the atoms necessary to complete a ketodiazine nucleus,  
Ar=o-, m- or p-arylene,  
X=acyl.

The ketodiazine nucleus may be for example 4-pyrimidone or 4-quinazolone.

Compounds containing a 4-quinazolone nucleus may be prepared as follows:

The sodium salt of anthranilic acid is condensed with o-, m- or p-nitrobenzoylchloride. The resulting amide is treated with acetic anhydride, thus loses a molecule of water and is converted into a nitrophenylbenzoxazine compound. This compound is converted with ammonium hydroxide and pyridine into nitrobenzoylanthranilamide which by boiling in diluted sodium hydroxide is converted into nitrophenylquinazolone. The latter is reduced with hydrogen and Raney nickel to the corresponding aminophenyl quinazolone which by condensation with  $\text{XCH}_2\text{COOC}_2\text{H}_5$  gives the desired coupler.

2

Thus meta- and para-nitrobenzoylanthranilic acid obtained according to M. Bogert, R. Gortner and C. Amend, J.A.C.S. 33 (1911), 952, may be converted into 2-(m- and p-nitrophenyl)benzoxazine according to the same authors. The corresponding o-compound may be obtained as follows: o-nitro-benzoylanthranilic acid obtained according to H. Meyer, Ann. 351 (1907), 273, may be converted into 2-(o-nitrophenyl)benzoxazine according to G. Schroeter and O. Eisleb, Ann. 367 (1909), 132.

These benzoxazines may be converted into meta- and para-nitrobenzoylanthranilamide as illustrated by the following example:

30 g. 2-m-nitro-phenylbenzoxazine are refluxed with 75 cm.<sup>3</sup> pyridine and 40 cm.<sup>3</sup> of concentrated ammonium hydroxide. After cooling, sucking off the precipitate and recrystallizing from a mixture of dioxane and water, the meta-nitrobenzoylanthranilamide, melting at 230° C. is obtained.

Likewise, p-nitrobenzoylanthranilamide, melting at 242° C., and o-nitro-benzoylanthranilamide, melting at 192° C., are obtained. These anthranilamides may be converted into quinolones. For this purpose, m-nitrobenzoylanthranilamide is refluxed with sodium hydroxide N. The reaction mixture is acidified with hydrochloric acid and the precipitate is recrystallized from dimethylformamide. Small yellow needles of 2-(m-nitrophenyl)quinolone, melting above 300° C., are obtained.

Likewise 2-(p-nitrophenyl)-quinolone, also melting above 300° C. and 2-(o-nitrophenyl)-quinolone, melting at 232° C., are obtained.

These nitrophenylquinolones may be reduced as follows:

2-(p-nitrophenyl)-quinolone is dissolved in a mixture of piperidine and water (equal parts by volume) and reduced in the presence of Raney nickel by hydrogen under a pressure of 30 kg. per sq. cm. and at 75° C. until the theoretical absorption of hydrogen has taken place. The reaction mixture is concentrated in vacuum and acidified with acetic acid. The 2-(p-amino-phenyl)-quinolone, melting above 300° C., precipitates.

2-(m-nitrophenyl)quinolone is reduced in sodium hydroxide N by hydrogen under a pressure of 3 kg. per sq. cm. at 50° C. in the presence of Raney nickel. The reaction mixture is acidified with hydrochloric acid. A precipitate is formed by addition of ammonium hydroxide. The resulting 2-(m-aminophenyl)quinolone melts at 251° C.

2-(o-nitrophenyl)quinolone is reduced in dimethylformamide in the presence of Raney nickel by hydrogen under a pressure of 70 kg. per sq. cm. at 70° C. The resulting 2-(o-aminophenyl)quinolone melts at 225-227° C.

From these aminophenylquinolones, couplers may be prepared as follows:

The said quinolones are refluxed in dimethylformamide together with an excess of 10-15% of beta-keto-ester. The resulting beta-keto-anilide precipitates, is washed with methanol and recrystallized from glycol-methyl ether or dimethylformamide.

In this way the following compounds, for example, were obtained:

(1) 2-(p-benzoyl-acetamino-phenyl)-4-quinolone, melting above 300° C.

(2) 2-(m-benzoyl-acetamino-phenyl)-4-quinolone, melting at 275-277° C.

(3) 2-(o-benzoyl-acetamino-phenyl)-4-quinolone, melting at 240-241° C.

- (4) 2 - [m - alpha - furoyl - acetamino)phenyl] - 4 - quinazolone, melting at 261-263° C.
- (5) 2 - [m - (alpha - thenoyl - acetamino)phenyl] - 4 - quinazolone, melting at 257-259° C.
- (6) 2 - [m - (p - anisoyl - acetamino)phenyl] - 4 - quinazolone, melting at 245° C.
- (7) 2 - (m - acetylacetamino - phenyl) - 4 - quinazolone, melting at 202-205° C.

The presence, during color development, of color couplers according to the present invention, may arise from adding to the developer a compound which differs from the color coupler only because in the active  $\text{CH}_2$  group one or two hydrogen atoms are replaced by a group capable of splitting off either before development occurs by the action of the alkali in the developing solution or during the color-development.

The aromatic amino compounds, which according to our invention are used as developing agents, comprise mono-, di- and tri-amino aryl compounds, particularly N:N-dialkyl-para-phenylene diamines and derivatives such as N:N-dialkyl-N'-sulphomethyl-para-phenylene diamines. As mono-amino developers may be mentioned amino-phenols and amino-cresols and their halogen derivatives, and also amino-naphthols.

The following example serves to illustrate the invention without, however, limiting the scope thereof.

An exposed photographic film strip coated with a silver halide emulsion layer is developed in a bath of the following composition:

#### Solution A

|                                              |     |
|----------------------------------------------|-----|
| Sodium hexa-meta-phosphate                   | 1   |
| Sodium sulphite (anhydrous)                  | 3   |
| N:N-diethyl-p-phenylene-diaminehydrochloride | 3   |
| Sodium sulphate (anhydrous)                  | 40  |
| Sodium carbonate (anhydrous)                 | 35  |
| Potassium bromide                            | 1.5 |
| Water to 900 cm. <sup>3</sup>                | 40  |

#### Solution B

|                                                        |     |
|--------------------------------------------------------|-----|
| Sodium hydroxide                                       | 1.5 |
| One of the couplers 1 to 7 prepared as described above | 1   |
| Water to 50 cm. <sup>3</sup>                           |     |

Before use, Solution B is added to Solution A and water is added to the resulting solution to 1,000 cm.<sup>3</sup>. The

developed image is rinsed for thirty minutes and the silver is bleached in the following bath:

|                                |    |
|--------------------------------|----|
| Potassium ferricyanide         | 50 |
| Potassium bromide              | 3  |
| Water to 1000 cm. <sup>3</sup> |    |

The image is rinsed again for ten minutes and then fixed for twenty minutes in the following bath:

|                                |     |
|--------------------------------|-----|
| Sodium thiosulphate            | 250 |
| Water to 1000 cm. <sup>3</sup> |     |

and again rinsed for thirty minutes.

A yellow image is obtained.

We claim:

1. Process for obtaining a colored photographic image, comprising developing an image consisting of a reducible silver salt with a color forming developer containing an N,N-dialkyl-para-phenylene diamine as a developing agent, and a quinazolone color coupler selected from the group consisting of 2-(benzoyl-acetamino-phenyl)-4-quinazolone, 2-[m-(p-anisoyl-acetamino)-phenyl]-4-quinazolone, 2 - (m-acetyl-acetamino-phenyl)-4-quinazolone, 2-[m-(alpha-furoyl-acetamino)phenyl]-4-quinazolone, and 2-[m-(alpha-thenoyl-acetamino)phenyl]-4-quinazolone.

2. Photographic developer containing an N,N-dialkyl-para-phenylene diamine as a developing agent, and a quinazolone compound as a color coupler, said quinazolone compound being selected from the group consisting of 2-(benzoyl-acetamino-phenyl)-4-quinazolone, 2-[m-(p-anisoyl-acetamino)phenyl]-4-quinazolone, 2 - (m-acetyl-acetamino-phenyl)-4-quinazolone, 2 - [m - (alpha-furoyl-acetamino)phenyl]-4-quinazolone, and 2-[m-(alpha-thenoyl-acetamino)-phenyl]-4-quinazolone.

3. Process for obtaining a colored photographic image, comprising developing an image consisting of a reducible silver salt with a color forming developer containing an N,N-dialkyl-para-phenylene diamine as a developing agent, and 2 - (benzoyl-acetamino-phenyl)-4-quinazolone as a color coupler.

4. Photographic developer containing an N,N-dialkyl-para-phenylene diamine as a developing agent, and 2 - (benzoyl-acetamino-phenyl) 4-quinazolone as a color coupler.

#### References Cited in the file of this patent

#### UNITED STATES PATENTS

|           |               |               |
|-----------|---------------|---------------|
| 2,500,487 | Craig         | Mar. 14, 1950 |
| 2,668,112 | De Cat et al. | Feb. 2, 1954  |